



US006071571A

# United States Patent [19]

Lerch et al.

[11] Patent Number: 6,071,571

[45] Date of Patent: Jun. 6, 2000

[54] **DOUBLE PORCELAIN-COATED GAS BURNER AND METHOD OF MAKING SAME**

[75] Inventors: Allan C. Lerch; Michael E. Tracey, both of Louisville, Ky.

[73] Assignee: **Porcelain Metals Corporation, Inc.**, Louisville, Ky.

[21] Appl. No.: 09/031,347

[22] Filed: **Feb. 26, 1998**

[51] Int. Cl.<sup>7</sup> ..... **B05D 1/10**; B05D 1/36; B05D 1/18

[52] U.S. Cl. ..... **427/475**; 427/374.2; 427/419.3; 427/419.4; 427/427; 427/435

[58] Field of Search ..... 427/419.3, 419.4, 427/430.1, 435, 443.2, 427, 374.2, 425; 428/432, 433; 264/214, 215; 431/328

## [56] References Cited

### U.S. PATENT DOCUMENTS

- 2,864,721 12/1958 King et al.  
3,922,138 11/1975 Biddle et al.  
3,930,062 12/1975 Nedeljkoric.  
3,959,866 6/1976 Biddle et al.  
4,009,302 2/1977 Biddle et al.  
4,519,770 5/1985 Kesselring et al.  
4,828,481 5/1989 Weil et al.  
4,878,837 11/1989 Otto.  
4,883,423 11/1989 Holowczenco.  
4,889,481 12/1989 Morris et al. .

5,104,309 4/1992 Krieger .  
5,147,201 9/1992 Xiona .  
5,165,970 11/1992 Schmidt et al. .  
5,248,251 9/1993 Dalla Betta et al. .  
5,368,475 11/1994 Suppiah et al. .  
5,455,011 10/1995 Kitto .

Primary Examiner—Fred J. Parker  
Attorney, Agent, or Firm—Middleton & Reutlinger; James R. Higgins, Jr.

[57]

## ABSTRACT

A two-step method to porcelain-coat an article is provided particularly useful for porcelain-coating a gas burner used in a gas-fired residential barbecue grill. A gas burner constructed from mild enameling-grade steel is dipped in a slip containing porcelain frit and manipulated so that the slip adequately coats and adheres to the interior surfaces of the burner. The porcelain-containing slip simultaneously coats and adheres to the peripheral “shoulders” and particularly to the interior “shoulders”, of the gas jet openings of the burner. A second coating of porcelain-containing powder is then applied, for example, electrostatically or by other conventional powder application techniques, to the exterior surfaces of the burner. The properties of the porcelain-containing powder of the second coating are adjusted for optimal coating properties. Then, the double coated gas burner is fired in a continuous furnace at a peak firing temperature of 1480° F. to 1550° F., with a target of 1530° F.±10° F. for about ten minutes, which adequately bonds the porcelain to the steel gas burner.

68 Claims, 3 Drawing Sheets







FIG. 2



FIG. 3



FIG. 4

**DOUBLE PORCELAIN-COATED GAS  
BURNER AND METHOD OF MAKING SAME**

**FIELD OF THE INVENTION**

The present invention relates to coating gas burners with a heat-resistant coating, and particularly to providing a double coating of porcelain on gas burners used in residential gas-fired grills, and a method of applying the double porcelain coating to such gas burners.

Residential gas-fired "barbecue" grills have gained wide popularity in recent years as consumers have indicated a purchasing preference for gas-fired grills in increasing numbers over charcoal fired grills. Such gas-fired grills are of well-known construction and usually are provided with a replaceable or rechargeable reservoir of fuel, such as propane, which is fed to a gas burner located within a cooking chamber of the grill. The gas burner is the most failure-prone component of the typical gas-fired grill. First of all, the barbecue grill is often stored outside for long periods of time, thereby subjecting the burner to atmospheric attack in a wide variety of ambient conditions. Further, the combustion characteristics of the gas used in most residential gas grills produce thermal reactions which cause the gas jets to burn out, or cause thermal stresses to appear which crack the burner and render it useless, or even dangerous. Consequently, the average life of a typical gas burner of a gas-fired residential barbecue grill is about two years, or even less.

Heretofore, burners of residential gas-fired barbecue grills have been fabricated of stainless steel. However, because of the above-described harsh environment and combustion characteristics, corrosion causes failure to occur at the gas jet orifices and burner seams. One known method to reduce the thermal damage to gas burners is to porcelain-coat the gas burner, and some attempts have occurred recently to porcelain coat such burners. These attempts have increased the life of the gas jet orifices, but have not been successful in protecting the interior surfaces of the combustion chamber of the gas burner. Consequently, the life of a gas burner for residential barbecue grill is still problematically low.

There are several patents in the field of coating gas burners for residential or commercial stoves. However, the teachings of those patents cannot be successfully translated to the particular configurations or ambient operational conditions presented by a typical gas burner for a residential barbecue grill. Indeed, presently-known methods of porcelain coating articles have proven to be inadequate to provide a sufficient porcelain coating on all critical surfaces of the gas burner, including the interior surfaces of the gas combustion chamber, the exterior surfaces of the gas burner and, particularly, the interior peripheries or "shoulders" of the gas jet orifices of the gas burner.

Accordingly, the present invention is a novel method to porcelain coat a gas burner for a gas-fired residential barbecue grill, and the double porcelain-coated burner made by such method.

**SUMMARY OF THE PRESENT INVENTION**

Briefly stated, the present invention is a two-step method to porcelain-coat an article, particularly useful in porcelain-coating a gas burner used in a gas-fired residential barbecue grill. First, the gas burner, which due to the present invention may now be made of mild enamelling-grade steel, is dipped in a slip containing porcelain frit and manipulated so that the slip adequately coats and adheres to the interior surfaces of the burner. At this same time, the porcelain-containing slip

also coats and adheres to the peripheral "shoulders", particularly the interior "shoulders", of the gas jet openings of the burner. Second, an acid-resistant powder containing porcelain frit is electrostatically applied to the exterior surfaces of the burner. Then, the slip-coated and powder-coated gas burner is fired in a continuous furnace at a peak firing temperature of 1480° F. to 1550° F., with a target of 1530° F.±10° F. for about ten minutes, which adequately bonds the porcelain to the steel gas burner.

Using this two-step coating process results in a gas burner that has an adequate porcelain coating applied to all critical surfaces of the gas burner, the exterior surfaces, the interior surfaces of the gas combustion area and the interior and exterior "shoulders" of the gas jet orifices. The porcelain coating(s) provided in this manner are thereby resistant to external ambient attack and also to internal thermal attack from the combustion process. This provides a protective surface at a critical failure point of the gas jet, thereby extending, to a surprising degree, the life of a gas burner made according to the present invention. For example, whereas the average life of gas burners used in residential gas-fired barbecue grills is about 2 years, more or less, one national manufacturer of residential gas-fired barbecue grills is now offering a limited five-year warranty on porcelain-coated gas burners made according to the present invention.

**BRIEF DESCRIPTION OF THE DRAWINGS**

FIG. 1 is a perspective view of the porcelain coated gas burner of the present invention, with a cut-away portion revealing the interior thereof;

FIG. 1A is an exploded view of a portion of FIG. 1;

FIG. 2 is a cross-sectional view of the gas burner, taken along line 2—2 of FIG. 1;

FIG. 3 is a cross-sectional view of the gas burner, taken along line 3—3 of FIG. 1; and

FIG. 4 is a Flow Chart of the Steps of the Preferred Embodiment of present invention.

**DESCRIPTION OF THE PREFERRED  
EMBODIMENT**

Referring now to FIGS. 1, 2 and 3 there is presented a gas burner 10 for use in a gas-fired residential barbecue grill (not shown) made according to the present invention, with an exterior porcelain coating 12 on the exterior surfaces of the burner, and interior porcelain coating 14 on the interior surfaces of the burner, and also a porcelain coating 15 on the interior and exterior "shoulders" 17 of the gas jets 18 of the burner.

A typical gas burner 10 for a residential barbecue grill is generally oblong, with two combustion chambers 16 each having a plurality of gas jet orifices or apertures 18 on the upper portion of the exterior surface 16e of each combustion chamber 16. The gas burner 10 is mounted by means of mounting surface 22 having mounting aperture 24 therein to receive an appropriate fastener (not shown) to mount the burner 10 in an appropriate cooking position in the grill. Cooking gas, usually propane, is provided from a gas tank (not shown) and fed into the interior 16i of each combustion chamber 16 through a gas inlet port 20 in each combustion chamber 16. The cooking gas is ignited within the interiors 16i of combustion chambers 16, and gas flames (not shown) emit through the orifices 18 of combustion chambers 16 to provide a row of cooking heat to the gas grill.

Examination of the cut-away portion of FIG. 1 as well as FIGS. 2 and 3, reveals that an interior porcelain coating 14

is provided on the interior surfaces of the burner. A key feature of the gas burner made according to the method of the present invention is that an adequate porcelain coating 15 is provided on the both the interior and exterior peripheral "shoulders" 17 of the gas jet orifices 18.

Referring additionally to FIG. 4 shows the preferred process to make the porcelain-coated gas burner 10 of the present invention. First, the raw, uncoated gas burner 10, which can now be made of enamelling grade steel, is pressure washed with an alkaline cleaner to remove mill oils, drawing compounds and other residue from the surfaces of the steel. While any number of alkaline cleaners would be adequate, we have found that a cleaner "TexoLite MAC" available from Texo, Inc. of Cincinnati, Ohio performs satisfactorily.

Next, the washed uncoated burner 10 is dipped into a relatively thin porcelain frit slurry. The slurry is made according to conventional wet porcelain practices. While any number of wet porcelain frit slurries would likely produce acceptable results, we have found the following formulation to produce satisfactory results:

TABLE I

| General Composition of Porcelain Wet Coat for Slip |         |
|----------------------------------------------------|---------|
| Glass frits                                        | 90-100% |
| Clays                                              | 0-10%   |
| Electrolytes                                       | 0-0.5%  |
| Oxides                                             | 0-1.0%  |

A particular formulation of wet coat that has provided satisfactory results is:

TABLE II

| Charge of Wet Porcelain Slip |                                |
|------------------------------|--------------------------------|
| 100 lbs                      | Mixture of 3 ground coat frits |
| 8 lbs                        | Mixture of 3 clays             |
| 0.5 lbs                      | Mixture of 4 electrolytes      |
| 50 lbs                       | Water                          |

The ground coat frits utilized in the above formulation are Nos. 10506, 10508 and 10509 purchased from CV Materials, Ltd. of Urbana Ohio. The clays utilized are M-79 and M-16 grade clays, plus bentonite purchased from Pemco Corp. of Baltimore Md. The electrolytes used in the above formulation are boric acid, sodium aluminate, potassium carbonate and 2-2600 "Set-It HK". The boric acid, sodium aluminate and potassium carbonate are commercially available from a number of suppliers, and S-2600 "Set-It HK" is available from Pemco. In some cases, in addition to the above materials, it may be desirable to use tris nitro available from Pemco, or the like, to kill bacteria present in some waters. When we use such material, we use about 4-7 grams per 100 pounds in the above total charge of Table II.

It is known that the oxides of the above formulation are generally used to provide color to the porcelain coat. At present, we want the finished porcelain coat to be black, so we use five pounds of G635 or G621 black oxide available from Pemco in the total charge of Table II.

The foregoing ingredients are mixed with water in a standard wet ball mill containing high density alumina balls of 1" to 3" diameter and milled for approximately 3.5 hours, or until only about 6-8% of solids are retained on a 200 mesh (U.S. Series) screen. When emitted from the ball mill, the ball-milled slip has a specific gravity of about 1.7, but is

adjusted in a known manner to a specific gravity of about 1.59 to about 1.66, preferably about 1.63. This lower specific gravity is important, as is explained more fully below.

It is important that the wet coat porcelain slip be of a lower than normal specific gravity, in the range of about 1.59 to about 1.66. The lower specific gravity slip permits the slip to coat virtually all the interior surfaces 16*i* of the combustion chambers 16 of the gas burner, including the providing a porcelain coating 15 on the interior shoulders 17 of the gas jet orifices 18 of the combustion chambers 16. At present, we have found that a slip of a specific gravity of about 1.63 produces the best results. Also at present, we hand dip the cleaned raw burner 10 into the low specific gravity slip, including manipulating the burner to ensure maximum coating of the porcelain slip on the interior surfaces 14 and shoulders 15, produces the best results. Using the lower specific gravity slip produces a "pick up" rate of about 6 to about 14 grams per square foot of surface area, which results in a fired porcelain coating in the range of about 1.5 mils to about 2.5 mils on the interior surfaces 14 of the burner 10. We are confident that an appropriate automated dipping process would produce acceptable results, so long as the specific gravity of the wet coat slip were maintained within the above range or at the preferred specific gravity and the burner 10 were manipulated to provide target coating pick up thicknesses set forth herein.

After the burner 10 has been dipped into the low specific gravity wet coat slip, the exterior of the wet-coated burner 10 is cleaned with an air knife to ensure that the gas jet orifices 18 are not clogged, but at the same time that a sufficient shoulder coating 15 of wet coat slip remains on the periphery or shoulders 17 of the gas jet orifices 18. Then excess wet coat slip is removed from the exterior of the coated burner 10.

Next, the de-clogged burner 10 with excess slip removed (but with wet coat porcelain still coated on the interior 14 including with a retained shoulder/periphery coating 15 on the shoulders 17) is dried for about 5 to 8 minutes in a forced-air dryer at about 400° F., sufficient to present the exterior surfaces to receive an acid-resistant powder coat of porcelain. An infrared dryer could also be used, and it would likely require a shorter drying time.

The powder coat used in the present invention is No. 60103 EDS Powder available from CV Materials of Urbana Ohio, the composition of which is proprietary to CV Materials. The powder is electrostatically sprayed onto the exterior surfaces of the burner 10 in an understood manner, to produce a fired thickness of about 2.5 to about 5.5 mils. Exterior fired-on powder coatings of less than about 2.0 mils will tend to burn off, while powder coatings greater than 5.5 mils will have a tendency to spall, both of which could separately lead to premature failure of the burner 10.

The wet-coated and powder-coated burner 10 is then fired in a continuous furnace to a peak temperature of about 1480° F. to about 1550° F., with a preferred peak firing temperature of 1530° F.±10° F., for about five minutes a peak temperature. As is generally understood in the porcelain enameling industry, in a continuous furnace, to-be-fired articles (e.g., the wet-coated and powder-coated burners 10) are suspended by hooks or the like from a heat-resistant wire or chain which traverses the length of the furnace. The furnace contains heating zones of different temperatures throughout the traversed length of the furnace, such that the temperature of entrance of the furnace is generally at ambient temperature and zones of increased temperature are provided including a peak temperature firing zone, followed by zones of

decreased temperature until the exit portions of the furnace are generally at ambient temperature. In the present invention, the firing cycle is such that the double-coated burners **10** traverse through the furnace at a line speed of about 10-20 feet per minute, such that the double-porcelain coated gas burners **10** are exposed to the peak firing temperature for about five minutes.

The firing of the double-coated burner **10** thermally bonds the porcelain to the steel in a well-understood manner, with the result that the finished porcelain-coated gas burner **10** has adequate porcelain coating on the exterior surfaces **12**, the interior surfaces **14** and the shoulder or peripheral surfaces **15**.

While in the foregoing specification this invention has been described in relation to specific preferred embodiments thereof, and many details have been set forth for the purpose of illustration, it will be apparent to those skilled in the art that the details are provided only by way of example, and the invention is not intended to be limited to the specific embodiments set forth herein, but rather is susceptible to additional embodiments, and that certain of the details described herein can be varied considerably without departing from the basic principles or scope of the invention.

Having thus described the invention with the detail and particularity required by the Patent Laws, what is desired to be protected by Letters Patent is set forth in the following appended claims.

We claim:

1. A method of coating an article having orifices therein with heat resistant porcelain material on its interior and exterior surfaces, comprising the steps of:

providing an article having apertures therein to be coated; providing a porcelain-containing aqueous slip; immersing said article in said slip to coat the interior and exterior surfaces and the peripheral shoulders of said orifices;

removing excess slip from said apertures and said exterior surface while retaining a coating of said porcelain-containing slip on the shoulders of said orifices;

40 applying a porcelain-containing powder coating to said exterior surface and to said shoulders of said orifices; firing said article at sufficient temperatures to thermally bond the porcelain of said porcelain-containing slip to said interior surfaces, and thermally bond the porcelain of said porcelain-containing powder to said exterior surfaces, and also provide a thermal bonded porcelain coating around said shoulders of said orifices to form a porcelain-coated article.

2. The method of claim 1 when said article to be coated 50 is a gas burner.

3. The method of claim 2 wherein said gas burner is comprised of enamelling grade steel.

4. The method of claim 3 including the additional step of alkaline cleaning said steel gas burner prior to immersing 55 same in said porcelain-containing slip.

5. The method of claim 4 wherein said porcelain-containing slip comprises glass frit of about 90 to about 100%, clays of about 0 to about 10%, electrolytes of about 0 to 0.5 percent and oxides of about 0 percent to about 0.1 percent mixed in water and is provided at a specific gravity 60 in the range of about 1.59 to about 1.66.

6. The method of claim 4 wherein said porcelain-containing slip comprises glass frit of about 90 to about 100%, clays of about 0 to about 10%, electrolytes of about 0 to 0.5 percent and oxides of about 0 percent to about 0.1 percent mixed in water and is provided at a specific gravity 65

in the range of about 1.59 to about 1.66 is provided at a specific gravity of about 1.63.

7. The method of claim 4 wherein said coating of said porcelain-containing slip is provided on the interior surfaces of said burner at a thickness in the range of between 1.5 mils to about 2.5 mils.

8. The method of claim 4 wherein said coating of said porcelain-containing slip on the interior surfaces of said gas burner is provided at a pickup rate in the range of about 6 to about 10 14 grams per square foot.

9. The method of claim 4 wherein said coating of said porcelain-containing slip on the interior surfaces of said gas burner is provided at a pickup rate in the range of about 9 grams per square foot.

10. The method of claim 4 wherein said porcelain-containing powder is electrostatically applied to said exterior surfaces of said burner to produce a fired thickness in the range of between 2.5 to about 5.5 mils.

11. The method of claim 4 wherein said firing occurs at a peak temperature in the range of about 1480° F. to about 1550° F.

12. The method of claim 4 wherein said firing occurs at a peak temperature in the range of about 1520° F. to about 1540° F.

13. The method of claim 4 wherein said firing occurs at a peak temperature of about 1530° F.

14. The method of claim 4 wherein said firing occurs in a continuous furnace, wherein said coated articles are traversed through said furnace while suspended from a traveling line which travels through said furnace at a speed of about 10 to about 20 feet per minute, whereby said coated burners are subjected to the peak firing temperature for about five minutes.

15. A method of coating an article having interior surfaces, exterior surfaces, and orifices therein with heat resistant porcelain material comprising the steps of:

a) providing a first aqueous solution with a specific gravity in the range of 1.55 to 1.66 containing a first heat resistant porcelain material;

b) immersing a metal gas burner article having orifices therein to be coated in said first aqueous solution so as to provide a pickup coating in the range of about 6 to about 14 grams per square foot of surface area of said aqueous solution on the interior and exterior surfaces of said article, and on shoulder surfaces of said orifices;

c) removing any excess of said aqueous solution from, and drying the exterior surface of, said article;

d) spraying a powder containing second heat-resistant porcelain material onto the exterior surface of said article;

e) subjecting said article containing said first heat-resistant material and said second heat-resistant material to a temperature in the range of 1480° F. to 1550° F. to thermally bond said first and second heat-resistant materials to said article; and

f) cooling said thermally bonded article to form a porcelain coated article having porcelain coating on the interior surfaces, exterior surfaces, and shoulder surfaces of said orifices.

16. The method of claim 15 including the additional step of alkaline cleaning said article prior to immersing it in said aqueous solution.

17. The method of claim 16 wherein said article is a steel gas burner.

18. The method of claim 17 wherein said first heat resistant material is a porcelain-containing slip comprised of

90 to 100 percent glass frit, 0 to 10 percent clays, 0 to 0.5 percent electrolytes and 0 to 0.1 percent oxides mixed in water resulting in a specific gravity of said slip of between 1.59 and 1.66.

**19.** The method of claim 17 wherein the selected pickup 5 of said aqueous solution on said interior surfaces is in the range of about 6 to about 14 grams per square foot.

**20.** The method of claim 17 wherein said second heat-resistant material is a porcelain-containing powder electrostatically sprayed onto said exterior surfaces to produce a 10 fired thickness of about 2.5 to about 5.5 mils.

**21.** The method of claim 17 wherein said selected elevated temperature is in the range of about 1480° F. to about 1550° F.

**22.** The method of claim 17 wherein said selected 15 elevated temperature is in the range of about 1540° F.

**23.** The method of claim 17 wherein said burner is subjected to peak elevated temperature for about five minutes.

**24.** The method of claim 17 wherein said porcelain is 20 thermally bonded to said interior surfaces and said exterior surfaces and said periphery of said shoulders of said orifices of said burner.

**25.** A method of porcelain coating the interior and exterior 25 surfaces and orifice surfaces of a steel gas burner comprising the steps of:

- a) providing a pre-formed steel gas burner having orifices therein;
- b) alkaline washing said gas burner to clean the surfaces 30 of said gas burner;
- c) providing a porcelain-containing slip of specific gravity in the range of about 1.59 to about 1.66, said slip comprising about 90 to about 100 percent glass frit, about 0 to about 10 percent clays, about 0 to about 0.5 percent electrolytes and about 0 to 1.0 percent oxides mixed in water;
- d) hand dipping said alkaline-washed gas burners in said slip and manipulating said burner in said slip so as to provide a coating of same slip on the peripheral shoulders of said orifices and the interior surfaces of said gas burner of a fired thickness in the range of about 1.5 to about 2.5 mils;
- e) removing excess slip from the orifices of said gas burner, leaving said slip coated on the peripheral shoulders of said orifices;
- f) removing excess slip from the exterior surfaces of said burner and drying said exterior surfaces;
- g) electrostatically spraying an acid-resistant porcelain-containing powder to said dried exterior surfaces of 50 said gas burner to provide a fired thickness of about 2.5 to about 5.5 mils; and
- h) firing the coated and sprayed burners in a continuous furnace, wherein said coated and sprayed burners are suspended on a line traveling through said furnace at a line speed of about 20 feet per minute and where the coated and sprayed burners are subjected to a peak firing temperature of about 1520° F. to about 1540° F. for about five minutes to thermally bond said porcelain of said porcelain-containing slip and said porcelain-containing powder to said interior surfaces and said exterior surfaces and said peripheral shoulders of said orifices of said burner to form a porcelain coated steel gas burner.

**26.** A method of porcelain coating a steel gas burner 65 having interior and exterior surfaces, and gas jet orifices therein, comprising the steps of:

a) dipping the burner in a porcelain-containing slip of a specific gravity in the range of 1.59 to 1.66 to coat at least the interior surfaces and shoulders of said gas jet orifices with porcelain slip;

b) applying a coating of porcelain-containing powder to the exterior surfaces of said burner; and

c) firing said slip-coated interior surfaces, said slip-coated shoulders and said powder coated exterior surfaces to thermally bond said porcelain to said interior surfaces, said shoulders and said exterior surfaces to form a porcelain coated steel gas burner.

**27.** The method of claim 26 wherein said gas burner is comprised of steel.

**28.** The method of claim 27 wherein said selected specific gravity of said porcelain-containing slip is about 1.63.

**29.** The method of claim 27 wherein said porcelain-containing slip is applied to said interior surfaces to provide a fired thickness of about 1.5 to 2.5 mils.

**30.** The method of claim 27 wherein said coating is applied to said exterior surfaces in a fired thickness of about 2.5 to 5.5 mils.

**31.** The method of claim 27 wherein said burner containing said applied porcelain-containing slip and said porcelain-containing powder is fired at a peak temperature of about 1480° F. to about 1550° F. for about five minutes.

**32.** The method of claim 27 wherein said burner containing said applied porcelain-containing slip and said porcelain-containing powder is fired at a peak temperature of about 1520° F. to about 1540° F. for about five minutes.

**33.** The method of claim 27 wherein said burner containing said applied porcelain-containing slip and said porcelain-containing powder is fired at a peak temperature of about 1530° F. for about five minutes.

**34.** A method of porcelain coating a steel gas burner 35 having interior and exterior surfaces and gas jet orifices therein, comprising the steps of:

a) dipping the burner in a porcelain-containing slip of a specific gravity between about 1.59 to about 1.66 to coat at least the interior surfaces to a fired thickness of about 1.5 to about 2.5 mils and also to coat the peripheries of said gas jet orifices with porcelain slip;

b) applying a coating of acid resistant porcelain-containing powder to the exterior surfaces of said burner in a fired thickness of about 2.5 to about 5.5 mils; and

c) firing said slip-coated interior surfaces, said slip-coated aperture peripheries and said powder-coated exterior surfaces in a continuous furnace to a peak temperature of between about 1480° F. to about 1550° F. for about five minutes to thermally bond said porcelain to said interior surfaces, said peripheries and said exterior surfaces to form a porcelain coated steel gas burner.

**35.** A porcelain coated article made according to the 55 method of claim 1.

**36.** A porcelain coated article made according to the method of claim 2.

**37.** A porcelain coated article made according to the method of claim 3.

**38.** A porcelain-coated gas burner made according to the method of claim 4.

**39.** A porcelain-coated gas burner made according to the method of claim 5.

**40.** A porcelain-coated gas burner made according to the method of claim 6.

**41.** A porcelain-coated gas burner made according to the method of claim 7.

- 42.** A porcelain-coated gas burner made according to the method of claim **8**.
- 43.** A porcelain-coated gas burner made according to the method of claim **9**.
- 44.** A porcelain-coated gas burner made according to the method of claim **10**.
- 45.** A porcelain-coated gas burner made according to the method of claim **11**.
- 46.** A porcelain-coated gas burner made according to the method of claim **12**.
- 47.** A porcelain-coated gas burner made according to the method of claim **13**.
- 48.** A porcelain-coated gas burner made according to the method of claim **14**.
- 49.** A porcelain coated article made according to the method of claim **15**.
- 50.** A porcelain coated article made according to the method of claim **16**.
- 51.** A porcelain coated gas burner made according to the method of claim **17**.
- 52.** A porcelain coated gas burner made according to the method of claim **18**.
- 53.** A porcelain coated gas burner made according to the method of claim **19**.
- 54.** A porcelain coated gas burner made according to the method of claim **20**.
- 55.** A porcelain coated gas burner made according to the method of claim **21**.

- 56.** A porcelain coated gas burner made according to the method of claim **22**.
- 57.** A porcelain coated gas burner made according to the method of claim **23**.
- 58.** A porcelain coated gas burner made according to the method of claim **24**.
- 59.** A porcelain coated steel gas burner made according to the method of claim **25**.
- 60.** A porcelain coated gas burner made according to the method of claim **26**.
- 61.** A porcelain coated steel gas burner made according to the method of claim **27**.
- 62.** A porcelain coated steel gas burner made according to the method of claim **28**.
- 63.** A porcelain coated steel gas burner made according to the method of claim **29**.
- 64.** A porcelain coated steel gas burner made according to the method of claim **30**.
- 65.** A porcelain coated steel gas burner made according to the method of claim **31**.
- 66.** A porcelain coated steel gas burner made according to the method of claim **32**.
- 67.** A porcelain coated steel gas burner made according to the method of claim **33**.
- 68.** A porcelain coated steel gas burner made according to the method of claim **34**.

\* \* \* \* \*

UNITED STATES PATENT AND TRADEMARK OFFICE  
**CERTIFICATE OF CORRECTION**

PATENT NO. : 6,071,571  
DATED : June 6, 2000  
INVENTOR(S) : Lerch et al

It is certified that error appears in the above-identified patent and that said Letters Patent is hereby corrected as shown below:

Claim 6, col. 5, change "mised" to --mixed --;  
Claim 6, col. 6, line 1, change "aobut" to --about --;  
Claim 21, col. 7, line 13, change "elevanted" to --elevated--;  
Claim 24, col. 7, line 22, change "periphey" to --periphery--.

Signed and Sealed this

Seventeenth Day of April, 2001

Attest:



NICHOLAS P. GODICI

Attesting Officer

Acting Director of the United States Patent and Trademark Office